

Jan. 5, 1932.

K. L. SCOTT ET AL

1,839,345

METHOD OF HEAT TREATING MAGNET STEELS

Filed Jan. 18, 1930



Inventors:  
K. L. Scott  
A. L. Kirby  
M. R. Leach

By R. H. Whitfield Att'y.

## UNITED STATES PATENT OFFICE

KENNETH L. SCOTT, OF WESTERN SPRINGS, ARTHUR L. KIRBY, OF CICERO, AND MARION R. LEACH, OF CHICAGO, ILLINOIS, ASSIGNEES TO WESTERN ELECTRIC COMPANY, INCORPORATED, OF NEW YORK, N. Y., A CORPORATION OF NEW YORK

## METHOD OF HEAT TREATING MAGNET STEELS

Application filed January 18, 1930. Serial No. 421,686.

This invention relates to a method of heat treating magnet steels, and more particularly to a method of improving the magnetic properties of cobalt magnet steel.

5 An object of the invention is to provide a method whereby material improvements in electrical and magnetic properties may be imparted to magnet steels.

It is a well known fact that in the ordinary methods of heat treating magnet steel 10 wherein the steel is quenched in a medium at, or lower than, room temperature, there is a progressive change with time, subsequent to the hardening, of the coercive force and the residual induction. The coercive force decreases with time at a progressively slow rate 15 while the residual induction increases. Since these changes have, in the ordinary methods, occurred simultaneously, it has been assumed that they must occur simultaneously. However, this assumption has been proved incorrect in that the residual induction increases 20 as before while the coercive force is stabilized, when the steel is quenched in a heated medium of the proper quenching temperature.

In the general embodiment of the invention the magnet steel is heated uniformly to a temperature above the critical temperature, after which it is quenched in a medium 30 at a temperature higher than room temperature, so as to give the magnet steel a slow quench and affect the magnetic properties thereof, the temperature of the quenching medium varying relative to the temperature of the magnet steel when heated.

Further objects of the invention may be apparent from the following description, taken in conjunction with the accompanying 40 drawing, in which the single figure is a time chart illustrating the subsequent relative condition of the magnetic properties of the magnet steel.

This method consists in first heating a 45 magnet steel, such as chrome steel, or cobalt steel containing 20% to 40% cobalt, to a uniform temperature of 1750° F. The magnet steel is then quenched in an oil, salt, or other medium which is maintained at a temperature 50 higher than room temperature. The

temperature of the quenching medium ranges from 200° F. to 600° F. depending upon the magnet steel, as, for example, a cobalt steel containing approximately 36% cobalt is quenched in a medium having a temperature 55 of 500° F. This quenching of the magnet steel in the heated medium brings about a slow quenching and consequently the magnet steel has very high coercive force.

Such a result is illustrated in the drawing, 60 wherein the horizontal line 1 indicates time subsequent to the quenching of the magnet steel and is graduated according to days. The vertical line 2 indicates the magnetizing force of the magnet steel according to gilberts 65 per centimeter. The high and stable coercive force which is the result of the slow quenching of the 36% cobalt steel at a temperature of 500° F. is illustrated by line 3 showing a coercive force of approximately 70 275 which is retained stable. The residual induction of the treated 36% cobalt steel is illustrated by the line 4.

As is well known, high coercive forces are of particular advantage in permanent magnets, and with this method of improving the magnetic properties of the magnet steels not only exceptionally high but stable coercive forces are imparted to the magnet steels. This specific example has been given as one 80 embodiment of the invention, but other tests have been made wherein higher and stable coercive forces have been obtained. The heat-treating temperature of 1750° F. is the preferred temperature for magnet steel containing 20% to 40% cobalt but the heat-treating temperatures may vary depending upon the metallic characteristics of the magnet steel being treated.

During each heat-treatment of magnet steel the steel is heated to a temperature above the critical temperature, which of course varies with the composition of the material being treated. Furthermore, even though only two classes of steels have been disclosed, it should be understood that 85 this invention is not limited to only these two classes of steels, but may include any other steel desired.

While the invention has been described with reference to a particular embodiment 90

thereof, various modifications may be made therein without departing from the spirit and scope of the invention.

What is claimed is:

- 5 1. A method of heat treating magnet steels, which consists in heating a magnet steel to a temperature above the critical temperature, and quenching the magnet steel in a medium heated to a temperature ranging  
10 from approximately 200° F. to approximately 600° F.
- 15 2. A method of heat treating magnet steels, which consists in heating a magnet steel to a temperature of approximately 1750° F., and slowly quenching the magnet steel in a medium heated to a temperature ranging from approximately 200° F. to approximately 600° F.
- 20 3. A method of heat treating magnet steels, which consists in heating a magnet steel to a temperature above the critical temperature, and quenching the magnet steel in a heated medium having a temperature of approximately 500° F.
- 25 4. A method of heat treating magnet steels, which consists in heating magnet steel to a temperature of approximately 1750° F., and quenching the magnet steel in a heated medium having a temperature of approximately  
30 500° F.

In witness whereof, we hereunto subscribe our names this 10th day of January A. D., 1930.

KENNETH L. SCOTT.  
ARTHUR L. KIRBY.  
MARION R. LEACH.

40

45

50

55

60

65